

Patented Oct. 13, 1953

2,655,469

# UNITED STATES PATENT OFFICE

2,655,469

## METHOD OF REMOVING ACTIVE SULFUR FROM SULFURIZED ORGANIC COM- POUNDS

Allan Manteuffel, Union, George R. Cook, North-  
field, and William D. Gilson, Crystal Lake, Ill.,  
assignors to The Pure Oil Company, Chicago,  
Ill., a corporation of Ohio

No Drawing. Application May 31, 1951,  
Serial No. 229,276

6 Claims. (Cl. 202—46)

1

This invention relates to the purifying of organic compounds prepared by reacting an organic compound with a sulfurizing agent such as elemental sulfur or sulfur halides.

In the lubrication of machinery the inherent lubricity of mineral oils permits the use of these mineral oils per se in many applications. However, because of the mechanical complexity of modern machinery and the environment in which it is employed there are numerous instances in which these indigenous properties of mineral oil lubricants have to be supplemented by the use of extrinsic additive agents which are blended into the mineral oil to produce the desired lubricating composition. These additive agents, which may be single purpose or multifunctional, act as pour point depressants, oxidation inhibitors, rust preventives, oiliness carriers, E. P. agents and other uses. Compositionwise, both organic and inorganic compounds have been found applicable. One type of composition which has found ready use has been sulfurized organic compounds. The beneficial properties of sulfurized materials were quickly discovered, and as a result this type of material has been employed for a longer time than other types of additive agents. Sulfurized compounds are versatile in their nature and, depending upon the method of processing and the initial raw materials employed, may be used to prevent oxidation, to impart oiliness, to promote film strength, etc. The prior art relating to the sulfurization of organic compounds is well developed. The major portions of this art, however, are devoted to the utilization of various raw materials as starting agents as well as various processing means whereby the various types of sulfur compounds are prepared. The refining of the sulfurized compounds thus produced has also been developed but improvements have been overshadowed by the manipulative processes used in the preparation of the sulfurized compounds.

In general in the refining of sulfurized materials the art is concerned with the production of light colored end products as well as the production of non-corrosive materials. Depending upon the reason for employing a sulfurized material in a mineral oil composition, the chemically combined sulfur may be "loosely bound" in the compound or may be present in a more stable

2

form. This latter aspect is important particularly when sulfurized materials are used as additive agents in lubricants employed in environments which are susceptible to sulfur corrosion. This invention is specifically concerned with preparing these stable sulfur-containing compounds. A specific application of these stable sulfur-containing compounded lubricants is in the lubrication of internal combustion engines where modern design practice has required the use of special bearing alloys such as cadmium-silver, cadmium-nickel and copper-lead. In order to obviate the sulfur corrosion problems which might result in the failure of these particular type bearings it is necessary not only to remove the loosely bound sulfur but also to refine the sulfurized material after it has been prepared in order to remove other sulfurous corrosive agents that might be present in the reaction mixture. These compounds generally take the form of active sulfur materials such as unreacted sulfurization reagents and various other organic and inorganic corrosive sulfur-containing compounds which are formed in side reactions occurring during the sulfurization step.

Various methods have been proposed by the prior art to alleviate the problem caused by these corrosion-producing impurities. One such method which is quite generally adopted is a controlled method of sulfurization wherein the reaction temperature employed during the sulfurization is maintained between critical limits. By this method side reactions, decomposition of the oil and insoluble polymer formation are substantially avoided. Other methods consist in refining the sulfurized material in a purification process that follows the sulfurization step. The non-volatile weakly acidic, sulfur-containing corrosive materials contained in the sulfurized mixture are removed by treating the reaction mixture with a purification agent which removes the undesirable sulfurous constituents. This agent may be used either in solution or in a dry comminuted form. The refining process then is concluded by subjecting the semi-refined sulfurized reaction mixture to a steam distillation wherein any volatile non-desirable reaction products are removed from the reaction mixture. A consolidation of the purification and steam distillation steps into one step has apparently been

studiously avoided by the prior art investigators because it has been found that unless the teachings of this invention are followed emulsification problems occur which make the refining process and the separation of the refined sulfurized material more difficult. However, these emulsion difficulties may be overcome and a single step purification process carried out wherein both the volatile and the non-volatile unreacted materials and side reaction products are removed from the 10 reaction mixture by a combined purification-steam distillation refining process by correlating the type of purification reagent employed with the temperature at which steam distillation is conducted.

It is therefore the object of this invention to provide a method for purifying a sulfurized material without experiencing any difficulty due to the formation of emulsions during the refining process.

A further object is to provide a method for removing unreacted sulfur, loosely bound sulfur and undesirable sulfur-containing side reaction products from sulfurized terpenes.

In accordance with this invention the purification of sulfurized organic materials to remove any volatile or non-volatile unreacted materials or side reaction products is effectuated by means of a single step operation in which a dry purification agent is added to the sulfurized mixture, and this resulting mixture is subjected to steam distilling at substantially atmospheric pressure at a sufficiently elevated temperature, not less than about 250° F., to prevent accumulation of moisture within the distillation vessel to such an extent as to cause emulsification difficulties. By limiting the amount of moisture that is permitted to be present, the purification agents and the salts formed during purification never become sufficiently hydrated to allow emulsification to occur. Under the conditions extant during the steam distillation an equilibrium is reached between these salts and the moisture from the steam so that as the purification reaction progresses, a dark viscous solution of a hydrated mixture of the purification agent and sulfurous impurities collects on the bottom of the distillation vessel. Enough moisture must be present during the purification process so as to allow intimate contacting of the purification agent with the sulfurized material through the turbulence provided by the steam distillation yet insufficient to cause emulsification.

This objective is obtained according to the present invention by employing a controlled temperature during the distillation. While the process may be also carried out at subatmospheric or superatmospheric pressures it is necessary to employ an elevated temperature not less than that temperature which would be the equivalent of the 250° F. temperature used in carrying out the process at atmospheric pressure. The upper limit in the distillation temperature is dictated by the temperature at which the sulfurized compound will be decomposed. For example, when treating a sulfurized terpene appreciable decomposition occurs at temperatures above about 350° F. releasing active sulfur which provides a corrosive environment.

It is to be noted at this point that the purification process employed by the present invention is not entirely a neutralization reaction. In contradistinction the greater part of the purification reaction essential to the present invention relies on the interaction between the sulfurous

5 impurities and the purification reagent to form organic and inorganic salts which are removed from the sulfurized material by forming a phase which varies in density from the density of the desired sulfurized material. This results in a phase separation which permits the facile recovery of the desired product.

6 The organic compounds which may be sulfurized and subsequently purified according to this invention are quite numerous. These materials include many types of unsaturated compounds which because of their high reactivity will react with various sulfurizing agents. Specific examples include various types of isoprenoid type materials, either per se or those obtained from such naturally occurring compositions as turpentine and pine oil, various naval stores products such as rosins, hydrocarbons and hydrocarbon mixtures such as petroleum oils, as well as other organic materials which when sulfurized and blended into a mineral oil lubricating composition will impart beneficial properties thereto. The sulfurization reagents which are employed by this invention to form the desired sulfurized product may be either elemental sulfur, the sulfur halides such as sulfur chloride and sulfur monochloride, or the sulfides of phosphorus such as the sesqui- and pentasulfides. Although any conventional method of sulfurization may be carried out to produce the crude sulfurized mixture it is preferred to prepare the sulfurized mixture by controlling the temperatures employed during the sulfurization reaction. This method, which employs elemental sulfur as the sulfurization agent, is fully described by Smith in United States Patent 2,179,060. Therein is pointed out the advantages of maintaining the reaction at certain specified temperatures in order to obtain the most advantageous results. Specific methods for sulfurizing terpenes are also disclosed by Powers in United States Patent 1,926,648 and Holt in United States Patent 2,443,823. A method of sulfurization employing a phosphorus sulfide as the sulfurization agent is shown by Musselman in United States Patent 2,331,923. Other methods of sulfurization which may be employed to prepare the crude sulfurized material which is refined in accordance with the method described by this invention may also be found in the prior art.

7 In order that this invention may be more clearly understood the following example is illustrative of the preferred sulfurization method as well as the novel refining process employed in this invention.

Example 1.—75 parts of Dipentene #122, which is a commercially available mixture of various terpenoid constituents containing approximately 50% dipentene, 17% paracymene, and 14% paramenthane, as well as other active and inert terpene hydrocarbons obtained from the Hercules Powder Company were charged to the reaction vessel. While stirring, 25 parts of elemental sulfur were added at room temperature or at initial heating temperatures below 100° F. It should be noted that this initial heating temperature is preferred although it is not a critical factor in the instant invention. The reaction temperature was then raised to about 280° F. to 290° F. as quickly as possible at a maximum rate of about 10° F. per minute. The mixture was maintained at this temperature for 45 minutes to 1 hour. Special care was taken when the reaction temperature was between 280° F. and 290° F. A slow dissipation 85 of the heat of reaction eliminated an unde-

strable exothermic reaction which if uncontrolled would have raised the reaction mixture to about 360° to 370° F. with accompanying ebullition. After the heat of reaction was dissipated the temperature was raised slowly (1 to 2° F. per minute) to about 320° F. and maintained at that temperature for about 3 to 5½ hours.

This method of preparation, in accordance with the teachings of the Smith patent, cited supra, minimized the presence of undesirable side reactions. In spite of this precautionary technique there was still present in the reaction mixture various constituents which either exert a deleterious effect because of the corrosiveness of these particular constituents or a neutral effect evinced by the unreacted starting materials. It was therefore necessary to further refine the sulfurized mixture in order to prepare a marketable and useful product. It is to this end that this invention relates. After the sulfurization reaction was completed 5% by weight of a combination of dry comminuted sodium hydroxide and sodium sulfide was added to the reaction mixture. When these agents had been added the crude reaction mixture was then steam distilled. The foregoing specific reagents are only illustrative as other purification agents employed in this invention may consist of a combination of various other alkali metal hydroxides and sulfides as well as alkaline earth sulfides and hydroxides. The desired amounts of purification reagents to be employed are dependent upon the nature of the reactants and must be determined experimentally for each type of sulfurization reaction. In general, 5% by weight of each of the purification agents should be used although in some instances as little as 1.0% by weight may be effective. On the other hand quantities as high as 25% by weight may be required in exceptional cases. It has been found that the combination of sodium hydroxide and sodium sulfide will provide the preferred results. The purification reagents may be added to the sulfurized mixture as the mixture thereof or separately and sequentially. That is, initially one of the purification reagents either the hydroxide or sulfide may be added to the crude sulfurized mixture and the steam distillation carried out. The impurities removed by this reagent are separated in the form of a viscous liquid phase. The remaining reagent is then added to the semi-purified mixture and the steam distillation continued until a non-corrosive sulfurized product is obtained. To determine whether or not the sulfurized compound has been sufficiently refined the well known Copper Strip test described by Smith in United States Patent 2,179,066 may be employed. The percent by weight of distillate is also used as a criterion of completion of reaction since for a given molecular structure of raw material there is a definite quantity of sulfur which will remain in the preferred combination. With the aid of the ebullition or turbulence provided by the steam there is intimate contact of the purification agent with the mixture. The purification reagents contained in the mixture react with the undesirable constituents of the mixture to form products which are readily separated. An equilibrium is also reached between the purification agents and the moisture from the steam so that as the purification reaction progresses a very dark viscous solution of the hydrated mixture collects at the bottom of the reaction flask. This can be drawn off and emulsification of the mixture avoided. To facilitate withdrawal of this hydrated mixture it

is preferred that a special reaction vessel with a bottom drain be provided so that as the viscous layer accumulates it can be drawn off without interrupting the steam distillation. It is essential that the temperature during steam distillation of the mixture be maintained above that temperature at which undesirable accumulations of moisture would result yet below that temperature at which the sulfurized material will appreciably decompose. For example, when the steam distillation is being conducted at atmospheric pressures a temperature above about 250° F. will be maintained. This controlled temperature feature minimizes the possibility of emulsion formation by preventing the accumulation of moisture within the mixture as the distillation progresses and limits the amount of moisture which can be maintained in equilibrium with the purification reagents. After the purification treatment is completed the dark viscous solution of the hydrated mixture is separated from the purified sulfurized compound. To insure removal of moisture and salt contamination from the sulfurized compound the product may be further improved by contacting the sulfurized material with a treating clay at a temperature of about 150° F. to remove residual inorganic salts, traces of deleterious sulfur compounds and traces of moisture. A clay having a 60/80 mesh is suitable. After clay contacting the finished sulfurized mixture will be clear and oil soluble in all proportions.

The results of the refining process described by this invention are seen in the tabulated data included in Table 1. In this table, which shows a comparison of the methods used for the removal of active sulfur from a terpene base, it will be seen that only when a combined purification reagent in the form of a mixture of dry comminuted sodium sulfide and sodium hydroxide was employed was there a decrease in the amount of sulfur which was active toward copper at the lower temperatures of 150° to 250° F. The results presented by this table show that only when the teachings of this invention are carried out in refining a sulfurized material is there shown a substantial reduction in the amount of total active sulfur present as well as a prevention of the emulsion difficulties which result when the prior art teachings are effectuated.

It is therefore seen that the method described by this invention provides a procedure for purifying a sulfurized organic compound to remove undesirable volatile and non-volatile impurities of a crude sulfurized reaction mixture by means of a single step refining process which circumvents any emulsification difficulties which would result from following the teachings of the prior art relating to the purification of sulfurized materials.

In the following claims the expression "organic materials" is intended to cover those compounds which will react with a sulfurization agent to form a sulfurized composition of matter in which sulfur is in tightly bound chemical combination and which in its crude form contains those undesirable non-volatile impurities such as unreacted elemental and loosely, chemically bound sulfur as well as other sulfurous compounds such as mercaptans, polysulfides, thio acids, etc. which are readily removed by treatment with an alkali metal hydroxide and an alkali metal sulfide as well as those volatile impurities which may be effectively removed by steam distillation.

7 TABLE I

Comparison of methods for active sulfur removal  
from terpene base

| Run | Percent sulfur in base after treat <sup>1</sup> | Method of active sulfur removal   |                      |                                      |                         | Emulsi-<br>fication | Percent of total sulfur active toward copper at temperature indicated |         |
|-----|-------------------------------------------------|-----------------------------------|----------------------|--------------------------------------|-------------------------|---------------------|-----------------------------------------------------------------------|---------|
|     |                                                 | Na <sub>2</sub> S wash, 30% sol'n | NaOH wash, 20% sol'n | Solid <sup>2</sup> Na <sub>2</sub> S | Solid <sup>2</sup> NaOH |                     | 150° F.                                                               | 250° F. |
| 1.  | 37.5                                            |                                   |                      |                                      |                         | Yes                 | 0                                                                     | 54      |
| 2.  | 34.3                                            | Yes                               | Yes                  |                                      |                         | Yes                 | 3                                                                     | 30      |
| 3.  | 33.0                                            | Yes                               | Yes                  |                                      |                         | No                  | 0                                                                     | 66      |
| 4.  | 34.3                                            |                                   |                      | Yes                                  | Yes                     | No                  | 8                                                                     | 56      |
| 5.  | 34.7                                            |                                   |                      | Yes                                  | Yes                     | No                  | 0                                                                     | 29      |
| 6.  | 28.9                                            |                                   |                      |                                      |                         |                     |                                                                       |         |

<sup>1</sup> Samples analyzed after treat for active sulfur removal.<sup>2</sup> Added to mixture while steam distilling.

What is claimed is:

1. A method for purifying a crude sulfurized organic material which comprises steam distilling the crude sulfurized reaction mixture in the presence of a combination of non-aqueous alkalis selected from the group consisting of the alkali metal and alkaline earth metal hydroxides and non-aqueous sulfide from the group consisting of alkali metal and alkaline earth metal sulfides at a temperature sufficiently elevated so as to prevent a greater accumulation of water than is required to produce substantially equilibrium hydration conditions between the purification reagents and the moisture from the steam but below a temperature at which the desired sulfurized organic materials decompose, the proportions of said reagents being sufficient to react with the corrosive sulfurous constituents of said mixture, carrying out said distillation until the reaction between the said purification reagents and the said corrosive sulfurous constituents of the reaction mixture is completed and the removal of volatile constituents is effected, separating the resulting phases, and recovering a non-corrosive, non-volatile sulfurized mixture.

2. A method of refining a crude sulfurized organic material which comprises steam distilling the crude sulfurized reaction mixture in the presence of a non-aqueous mixture of an alkali metal hydroxide and an alkali metal sulfide at a temperature sufficiently elevated so as to prevent a greater accumulation of water than is required to produce substantially equilibrium hydration conditions between the purification reagents and the moisture from the steam but below a temperature at which the desired sulfurized organic materials decompose, the proportions of said reagents being sufficient to remove the corrosive sulfurous constituents of said mixture, carrying out said distillation until the reaction between the purification reagents and the corrosive sulfurous constituents of the reaction mixture is completed, separating the resulting phases, and recovering a non-corrosive sulfurized material.

3. A method for producing a relatively non-volatile, non-corrosive, sulfurized organic material by steam distilling in the presence of a combination of non-aqueous purification reagents consisting of a hydroxide and a sulfide of an alkali metal which comprises initially carrying out the steam distillation in the presence of a purification reagent selected from the group consisting of hydroxides and sulfides of an alkali metal, separating the resulting phases, recovering a semi-purified sulfurized material, continuing the said distillation in the presence of an added proportion of the remaining purification reagent, separating the resulting phases and recovering a non-corrosive, non-volatile sulfurized mixture.

proportion of the remaining purification reagent, separating the resulting phases and recovering a non-corrosive, non-volatile sulfurized material, said distillations being carried out at a temperature sufficiently elevated as to prevent a greater accumulation of water than is required to produce substantially equilibrium hydration conditions between the purification reagents and the moisture from the steam but below a temperature at which the desired sulfurized organic materials decompose.

4. A method for producing a relatively non-volatile, non-corrosive, sulfurized organic material by steam distilling in the presence of a combination of non-aqueous purification reagents consisting of a hydroxide and a sulfide of an alkaline earth metal which comprises initially carrying out the steam distillation in the presence of a purification reagent selected from the group consisting of hydroxides and sulfides of an alkaline earth metal, separating the resulting phases, recovering a semi-purified sulfurized material, continuing the said distillation in the presence of an added proportion of the remaining purification reagent, separating the resulting phases and recovering a non-corrosive, non-volatile sulfurized material, said distillations being carried out at a temperature sufficiently elevated as to prevent a greater accumulation of water than is required to produce substantially equilibrium hydration conditions between the purification reagents and the moisture from the steam but below a temperature at which the desired sulfurized organic materials decompose.

5. A method of purifying a crude sulfurized isoprenoid material which comprises steam distilling the crude sulfurized isoprenoid reaction mixture in the presence of a combination of non-aqueous purification reagents consisting of a hydroxide and a sulfide of an alkali metal at a temperature sufficiently elevated so as to prevent a greater accumulation of water than is required to produce substantially equilibrium hydration conditions between the purification reagents and the moisture from the steam but below a temperature at which the desired sulfurized organic materials decompose, the proportions of said reagents being sufficient to remove the corrosive sulfurous constituents of said mixture, carrying out said distillation until the reaction between the purification reagents and the corrosive sulfurous constituents of the reaction mixture is completed and the removal of the volatile constituents is effected, separating the resulting phases, and recovering a non-corrosive, non-volatile sulfurized material.

6. A method of refining a sulfurized terpene

which comprises steam distilling the crude sulfurized terpene reaction mixture at substantially atmospheric pressure and at a temperature between about 250° F. and 350° F. in the presence of added amounts of a purification reagent consisting of a mixture of sodium sulfide and sodium hydroxide, carrying out said distillation until the reaction between the corrosive sulfurous constituents of said reaction mixture and the purification reagent is completed and the removal of the volatile constituents is effected, separating the resulting phases and recovering a

5 relatively non-volatile, non-corrosive sulfurized terpene.

ALLAN MANTEUFFEL,  
GEORGE R. COOK,  
WILLIAM D. GILSON.

References Cited in the file of this patent  
UNITED STATES PATENTS

| 10 Number | Name         | Date          |
|-----------|--------------|---------------|
| 2,443,823 | Holt -----   | June 22, 1948 |
| 2,445,983 | Watson ----- | July 27, 1948 |